

1,566,265

Dec. 22, 1925.

F. L. ANTISELL

PROCESS OF PRODUCING ELECTROLYTIC COPPER

Filed Jan. 11, 1922



Witness:

Harold Brockman

INVENTOR  
Frank L. Antisell

BY  
Cornelius P. Billings

ATTORNEY

## UNITED STATES PATENT OFFICE.

FRANK LINDEN ANTISELL, OF PERTH AMBOY, NEW JERSEY.

## PROCESS OF PRODUCING ELECTROLYTIC COPPER.

Application filed January 11, 1922. Serial No. 528,428.

*To whom it may concern:*

Be it known that I, FRANK LINDEN ANTISELL, a citizen of the United States, and a resident of Perth Amboy, county of Middlesex, State of New Jersey, have invented certain new and useful Improvements in Processes of Producing Electrolytic Copper, of which the following is a specification.

My invention concerns the electrodeposition of copper from aqueous solutions and it has for its object an improved process for conducting the electrolysis, whereby the copper deposited upon the cathode is of a quality superior to that obtained heretofore, having a greater copper content and a reduced quantity of impurities.

In carrying out the electrolysis of copper sulphate solutions as usually practiced in the copper refining industry, it is customary to employ an electrolyte which contains approximately three per cent copper and twelve per cent free sulfuric acid. In addition to the copper and acid such a solution as used in practice contains also a certain percentage of impurities, such as iron, alumina, selenium, etc.

Solutions of the above composition have been found to be the most satisfactory in view of the electric current carrying capacity of the copper ion and of the sulfuric acid ion or (sulphron  $\text{SO}_4$ ). During the electrolysis the  $\text{SO}_4$  ion dissolves copper at the anode, while at the same time the copper ion is deposited at the cathode. As the electrolysis proceeds, there results an impoverished film of electrolyte on the surface of each of the electrodes. The amount and thickness of the said impoverished film depends upon various conditions, such as the composition of the electrolyte, the temperature of the solution, the impurities contained therein, the amount of current passing through the electrolyte, the surface tension of the electrodes, and other factors.

With very low current densities the concentration of the positive and negative ions at the surface of the electrodes is low, and therefore the migration of the copper ions and the sulfuric ( $\text{SO}_4$ ) ion to their respective electrodes can continue, only slightly undisturbed. However, even at low current densities a tendency to polarization develops at the cathode, which precludes the possibility of producing dense deposits of

copper when current densities are used which are practically reasonable. As the current density is increased, the film of impoverished electrolyte at the cathode becomes greater, owing to the fact that the copper is removed at a great ratio, while the above mentioned impurities and copper which are present in the solution act as a concentration diaphragm which interferes with the rapid transfer of the sulfuric ( $\text{SO}_4$ ) ion to the anode. This phenomenon, in addition to the surface tension of the cathode, results in a film of impoverished electrolyte which is considerably greater at the lower edge of the cathode than at the top. As the result of this change in the electrolyte, free hydrogen is generated and hydrogen sulfid liberated and amorphous copper and hydrogen are set free at the cathode and incorporated with the metallic copper deposited thereon. The copper deposited under such conditions, while of relatively high purity, is mechanically in a strained condition, which condition manifests itself in the appearance of twinned crystals. In addition it also contains amorphous copper and hydrogen.

I have found that copper deposits having improved physical and metallurgical characteristics will be obtained by properly regulating the electrolyzing current, while the electrodes are submerged in the electrolyte, so as to remove the impressed electro-motive force (E. M. F.) and permit the counter electro-motive force (C. E. M. F.) to migrate the  $\text{SO}_4$  ion to the anode, and at the same time permit the migration of the copper ion from the anode to the cathode. The current is thus maintained at the instant of reduction of the impressed E. M. F. due to the concentrated cell action at the electrodes.

By stopping the flow of the current through the electrolyzing tank during the cycle, the amount of copper deposited will be lessened, but this loss is more than compensated for by the gain in physical and metallurgical characteristics of the copper deposit. When proceeding in such a manner I obtain deposits of dense electrolytic copper, free from twinned crystals and amorphous deposits of copper or hydrogen. I have found that good results are obtained by using twenty cycles per minute

with an open circuit for substantially twenty per cent per cycle, so that the impressed current in any particular period of time is established for substantially eighty 5 per cent of that time.

In carrying out my invention I preferably use an apparatus which is shown conventionally and diagrammatically in the accompanying drawing:

10 Fig. 1 of the said drawing represents an installation by means of which my improved process may be carried out.

Fig. 2 represents a plan view of the mechanical switching device.

15 Like numerals in the respective figures represent like parts.

As shown in Fig. 1, the installation comprises an electrolytic tank T filled with an electrolyte E, preferably consisting of a 20 copper sulfate solution. The said electrolytic tank T is provided in the usual manner with an anode A and a cathode C. The anode A is connected to the positive pole of a suitable electric generator G through the 25 circuit line L.

A mechanical switching device S is located in a tank O which is suitably filled with oil in order to reduce wear. This device may be in many forms, but a suitable current 30 and switch device may consist of a sheet of metal 10 disposed in the shape of a circle, which has a portion removed as at 10<sup>a</sup> as shown. A rotating brush 11 mounted on the shaft 12 and revolved by means of the 35 pulley 13, slides upon the said circular contact 10.

The negative line wire L' connects the cathode C with the rotating brush 11 and leads through L'' from the circular contact 40 10 back to the negative pole of the above mentioned electric generator G.

A condenser C' and a resistance R bridge the switching device between the lines L' and L'' as shown. It is desirable to mount 45 a plurality of brushes driven by a common shaft, and thus use a plurality of tanks through which the current is alternately

passed so that the load on the generator is more nearly constant.

It is thus evident that by varying the 50 speed of the rotating brush 11, I am enabled to obtain any desired number of interruptions of the electrolyzing current.

Having now described my invention, what I claim as new and desire to secure by Letters Patent is:

1. The process of electrolyzing cupriferous solutions which consists in carrying out the electrolysis in cycles, the electrolyzing current being impressed during each cycle 60 for a predetermined fraction thereof.

2. The process of electrolyzing cupriferous solutions which consists in carrying out the electrolysis in cycles, the electrolyzing current being impressed during each cycle 65 for a predetermined fraction thereof during the submersion of the electrodes.

3. The process of electrolyzing cupriferous solutions which consists in carrying out the electrolysis in cycles, the electrolyzing current being impressed during each cycle 70 for a predetermined fraction thereof, the impressed period being the longer.

4. The process of electrolyzing cupriferous solutions which consists in carrying out the electrolysis by impressing the electrolyzing current periodically at predetermined intervals.

5. The process of electrolyzing copper sulfate solutions which consists in carrying out the electrolysis in substantially twenty cycles per minute, the electrolyzing current being impressed during each cycle for substantially eighty per cent of the cycle period.

6. The process of electrolyzing cupriferous solutions which consists in carrying out the electrolysis by reversing the electrolyzing current periodically at predetermined intervals.

In witness whereof, I have hereunto set 90 my hand at the borough of Manhattan, city and State of New York, this 10th day of January, 1922.

FRANK L. ANTISELL.